# EUROPEAN PATENT SPECIFICATION

(11) **EP 4 130 338 B1**
(45) Date of publication and mention of the grant of the patent: **24.06.2026**
(21) Application number: 21781652.9
(22) Date of filing: 31.03.2021
(51) Int. Cl.: C23C 24/04, B05B 7/14, B05B 16/60, B05B 7/00

(54) **FILM FORMING APPARATUS AND FILM FORMING METHOD**
FILMBILDUNGSVORRICHTUNG UND FILMBILDUNGSVERFAHREN
DISPOSITIF DE FORMATION DE FILM ET PROCÉDÉ DE FORMATION DE FILM

(30) Priority: 31.03.2020 JP 2020065154
(43) Date of publication of application: 08.02.2023
(73) Proprietor: Osaka Gas Co., Ltd., Osaka-shi, Osaka 541-0046 (JP); National Institute of Advanced Industrial Science and Technology, Chiyoda-ku Tokyo 100-8921 (JP)
(72) Inventor: MANABE, Kyohei, Osaka-shi, Osaka 541-0046 (JP); HIGAKI, Katsuki, Osaka-shi, Osaka 541-0046 (JP); OHNISHI, Hisao, Osaka-shi, Osaka 541-0046 (JP); ECHIGO, Mitsuaki, Osaka-shi, Osaka 541-0046 (JP); SOGI, Tadayuki, Osaka-shi, Osaka 541-0046 (JP); AKEDO, Jun, Tsukuba-shi, Ibaraki 305-8560 (JP); AOYAGI, Rintaro, Tsukuba-shi, Ibaraki 305-8560 (JP); MATSUI, Hiroaki, Tsukuba-shi, Ibaraki 305-8560 (JP); SHINODA, Kentaro, Tsukuba-shi, Ibaraki 305-8560 (JP); TSUDA, Hiroki, Tsukuba-shi, Ibaraki 305-8560 (JP)
(74) Representative: LBP Lemcke, Brommer & Partner Patentanwälte mbB
(86) International application number: PCT/JP2021/013833
(87) International publication number: WO 2021/201099

(56) References cited:
- JP-A- 2007 246 937
- JP-A- 2008 075 149
- JP-A- 2008 184 647
- JP-A- 2010 221 161
- JP-A- 2011 084 787
- JP-A- 2013 170 309
- US-A1- 2009 191 349

## Description

### Technical Field

The present invention relates to a film forming apparatus and a film forming method for forming a film on a base material, and a formed film.

### Background Art

A technique called the aerosol deposition method (AD method) is a method for forming a film made of a metal oxide material on a base material without undergoing a high-temperature heat treatment such as sintering. The AD method is a method of forming a film on a base material by spraying a raw material powder made of minute particles such as a metal oxide from a nozzle toward the base material such as ceramic or plastic at about the speed of sound to crush and deform the minute particles using the energy obtained when the raw material powder collides with the base material.

As an apparatus used in the AD method, for example, a film forming apparatus described in Patent Document 1 has been proposed. The film forming apparatus described in Patent Document 1 includes an aerosol generating section that generates an aerosol obtained by mixing a raw material powder and a carrier gas, a nozzle that sprays the aerosol from a spray port, and the like, and the aerosol can be sprayed from the spray port of the nozzle toward the base material to form a film on the base material.

### Prior Art Documents

### Patent Document

Patent Document 1: Japanese Patent Application Laid-Open No. 2007-246937

Patent documents JP 2010 221161-A, JP 2008 075149 A and US 2009/191349 A1 disclose other AD apparatus and methods using the corresponding apparatus for making films from aerosols.

### Disclosure of the Invention

### Problem to be Solved by the Invention

In the AD method, the impact force of the minute particles colliding with the base material has a significant effect on the density of the film, and therefore in order to obtain a desired homogeneous film quality, the speed of the minute particles colliding with the base material needs to be controlled within an appropriate range. In particular, zirconia-based materials have high hardness, are less likely to undergo brittle deformation when colliding with a base material, and have a very narrow process window for film formation. For this reason, in order to form a homogeneous film, it is necessary to control the speed of the particles with high accuracy.

The film forming apparatus described in Patent Document 1 uses a nozzle with a small opening area and a diaphragm, or a nozzle with a rectangular flow path cross-section. However, when a nozzle with a small opening area and a diaphragm is used, the carrier gas component of the aerosol is rapidly accelerated at the ejection end of the nozzle, and therefore with a zirconia-based material that has a relatively high specific gravity, the particles cannot fully keep up with the acceleration of the carrier gas and collide with the base material at a low speed. As a result, there is a problem that a porous region having a low film density is generated, making it difficult to obtain a dense film. Also, if a nozzle with a rectangular flow path cross-sectional shape is used, there is a problem in that the gas flow is likely to be disturbed at the edges of the rectangle and the like, resulting in non-uniform gas speeds and consequently non-uniform particle speeds, and therefore it is difficult to obtain a homogenous film. Furthermore, if a nozzle with a relatively small opening area is used, there is a problem in that when a large amount of raw material powder is supplied for a long time, the raw material powder tends to accumulate inside the nozzle, and the accumulated raw material powder is ejected, whereby powder compact formation frequently occurs in which minute particles accumulate without being crushed or deformed at the time of collision with the base material, and thus defects occur in the film, making it unsuitable for mass production.

The present invention has been made in view of the above circumstances, and aims to provide a film forming apparatus and film forming method capable of stably supplying a large amount of ceramic raw material powder for a long time and forming a homogeneous and dense film, and a formed film.

### Means for Solving Problem

A characteristic configuration of the film forming apparatus according to the present invention for achieving the above object is a film forming apparatus for forming a film on a base material according to the appended claim 1.

According to the claim 1 configuration, the flow speed of the aerosol at the ejection end becomes uniform within the flow path cross-section due to making the cross-sectional shape of the ejection end of the aerosol transport path substantially circular. For this reason, a homogeneous and dense film can be formed on the base material. In addition, since the flow path cross-sectional area (area of the flow path cross-section) at the aerosol ejection end of the aerosol is 10 mm² or more, the flow path cross-sectional area at the ejection end is significantly larger than before, the ceramic raw material powder is less likely to accumulate inside the aerosol transport path, and a large amount of ceramic raw material powder can be stably supplied for a long time. Furthermore, by increasing the flow path cross-sectional area, the gas component of the aerosol is gradually accelerated in the flow path, and therefore, in particular, particles of even zirconia-based raw material powder that has a relatively large specific gravity are more likely to keep up with the acceleration of the gas. For this reason, it is possible to cause particles having a sufficient speed for obtaining a dense film to collide with the base material.

In another characteristic configuration of the film forming apparatus and film forming method according to the present invention, a distance from the ejection end of the aerosol transport path to the base material is 100 mm or less.

Since the aerosol ejected from the ejection end of the aerosol transport path spreads and is dispersed, the surface area of the film formed on the base material increases as the distance from the ejection end of the aerosol transport path to the base material increases. If the surface area formed on the base material increases, it is necessary to form the film over a wider surface area than the target film forming surface area when scanning the aerosol transport path or the base material to obtain a homogeneous film. Upon doing so, the amount of raw material powder used will increase, and there is a risk that the production cost will rise. According to the above characteristic configuration, due to the distance from the ejection end of the aerosol transport path to the base material being 100 mm or less, it is easier to suppress an increase in the production cost.

In another configuration of the film forming apparatus and film forming method a value obtained by dividing the area of the flow path cross-section at the ejection end of the aerosol transport path by a square of a distance between the ejection end of the aerosol transport path and the base material is 0.001 or more.

According to the above configuration, the value obtained by dividing the flow path cross-sectional area at the ejection end of the aerosol transport path by a square of a distance between the ejection end of the aerosol transport path and the base material is 0.001 or more, whereby the particle speed in the direction perpendicular to the base material at the time of colliding with the base material is less likely to vary, and therefore it is possible to suppress adhesion of a powder compact and formation of porosity, and it is possible to form a homogeneous film.

The film forming apparatus according to the present invention includes a processing chamber with an inner space in which at least a portion on a side of the ejection end of the aerosol transport path and the base material are arranged,
in which a flow path cross-section of the aerosol transport path at a processing chamber internal transport section located in the processing chamber has a substantially circular shape with an area of 10 mm² or more.

Also, the characteristic configuration of the film forming method according to the present invention includes arranging at least a portion on a side of the ejection end of the aerosol transport path and the base material in an inner space of a processing chamber, and
ejecting the aerosol toward the base material from the ejection end of the aerosol transport path in which a flow path cross-section at a processing chamber internal transport section located in the processing chamber has a substantially circular shape with an area of 10 mm² or more.

According to the above characteristic configuration, since the flow path cross-sectional area in the processing chamber internal transport section is substantially circular with a size of 10 mm² or more, the flowability of the aerosol is improved, and the ceramic raw material powder is less likely to accumulate in the aerosol transport path, and therefore a large amount of the ceramic raw material powder can be stably supplied for a long time.

In the characteristic configuration of the film forming apparatus and film forming method according to the present invention, the shape of the flow path cross-section at the processing chamber internal transport section corresponds to the shape of the flow path cross-section at the ejection end.

According to the above-described characteristic configuration, due to the shape of the flow path cross-section in the processing chamber internal transport section corresponding to the shape of the flow path cross-section at the ejection end, the flowability of the aerosol is improved, and the ceramic raw material powder is less likely to accumulate, and therefore a large amount of ceramic raw material powder can be stably supplied for a long time.

In another embodied configuration of the film forming apparatus and film forming method according to the present invention, a pressure in the processing chamber is 0.6 kPa or less.

Since the gas component of the aerosol rapidly decelerates and is dispersed to the surrounding area when it collides with the base material, there is a risk that it will be difficult for the particles affected by this to reach the base material at a sufficient speed. According to the above characteristic configuration, since the viscosity of the gas component of the aerosol is reduced, the particles are less likely to be affected by the gas motion when colliding with the base material, and therefore a denser and more uniform film can be formed.

In another characteristic configuration of the film forming apparatus and film forming method according to the present invention, the aerosol transport path is constituted by a straight pipe member.

According to the above characteristic configuration, the shape of the flow path cross-section is the same over the entirety of the aerosol transport path. For this reason, the flowability of the aerosol is improved, the ceramic raw material powder is less likely to accumulate, and a large amount of the ceramic raw material powder can be stably supplied for a long time.

In another embodied configuration of the film forming apparatus and film forming method according to the present invention, a density of particles constituting the ceramic raw material powder is 4.0 g/cm³ or more.

According to the above characteristic configuration, a homogeneous film can be formed based on the ceramic raw material powder constituted by particles having a density of 4.0 g/cm³ or more.

In another embodied configuration of the film forming apparatus and film forming method according to the present invention, the ceramic raw material powder is stabilized zirconia.

The inventor of the present application has confirmed through experiment that a homogeneous film can be formed when stabilized zirconia is used as the ceramic raw material powder.

In a characteristic configuration of the formed film according to the present invention for achieving the above object, the formed film is formed by the above-mentioned film forming apparatus or through the above-mentioned film forming method.

According to the above characteristic configuration, since the film is formed by a film forming apparatus or through a film forming method capable of forming a homogeneous and dense film, the formed film is homogeneous and dense.

### Brief Description of the Drawings

FIG. 1 is a diagram showing a configuration of a film forming apparatus according to an embodiment.
FIG. 2 is a view of an aerosol transport pipe according to the present embodiment viewed from a side of an ejection end.
FIG. 3 is a diagram showing a positional relationship between the aerosol transport pipe and the base material.
FIG. 4 is a diagram showing the ejection end of the film forming apparatus used in Comparative Example 1.
FIG. 5 is a diagram showing the ejection end of the film forming apparatus used in Comparative Example 2.
FIG. 6 is a diagram schematically showing a base material after film formation processing in Comparative Example 1.
FIG. 7 is a diagram schematically showing a base material after film formation processing in Comparative Example 2.

### Mode Of Embodying The Invention

Hereinafter, a film forming apparatus and a film forming method according to an embodiment of the present invention will be described with reference to the drawings.

### Film Forming Apparatus

As shown in FIG. 1, the film forming apparatus according to this embodiment includes a processing chamber 2, an aerosol generating section 6, an aerosol transport pipe 10 (aerosol transport path), a carrier gas feeding means 15, and the like.

The processing chamber 2 is an airtight housing. The inside of the processing chamber 2 is depressurized to a predetermined pressure (e.g., about 0.6 kPa) or less by discharging gas by a mechanical booster pump 3 and a vacuum pump 4 serving as exhaust equipment. Also, in the inner space of the processing chamber 2, a holding section 5 for holding a base material K to be subjected to the film forming processing and part of the aerosol transport pipe 10 are arranged.

The aerosol generating section 6 is a device that generates an aerosol by dispersing ceramic raw material powder in gas. In this embodiment, the aerosol generating section 6 is connected to a raw material powder supply section 7 via a raw material supply pipe S1. Also, the aerosol generating section 6 is connected to a carrier gas feeding pipe S2 and the aerosol transport pipe 10, which will be described later. Also, in the aerosol generating section 6, an aerosol is generated by mixing the ceramic raw material powder supplied from the raw material powder supply section 7 at a constant speed and the carrier gas fed by the carrier gas feeding means 15. The generated aerosol is fed to the aerosol transport pipe 10. Note that the time it takes to form a film having a target thickness can be shortened by increasing the supply speed of the ceramic raw material powder supplied from the raw material powder supply section 7 to the aerosol generating section 6, but if the supply speed is too high, pulsation will occur in the supply amount of the raw material powder, making it difficult to obtain a homogeneous film. On the other hand, if the supply speed is too slow, the film quality is improved, but the time required to complete film formation increases, and thus the manufacturing cost increases. For this reason, the supply speed of the ceramic raw material powder is preferably 1.5 to 30 g/min.

As shown in FIGS. 1 to 3, the aerosol transport pipe 10 has an ejection end 10a and a processing chamber internal transport section 10b (at least a portion on a side of the ejection end), and the ejection end 10a is disposed in the processing chamber 2 in such a manner as to oppose the holding section 5 in the processing chamber 2. The aerosol transport pipe 10 in the present embodiment is a cylindrical straight pipe member having a flow path cross-sectional area A1 (shaded portion in FIG. 3) with a predetermined inner diameter, and the end portion opposite to the ejection end 10a is connected to the aerosol generating section 6. That is, in the aerosol transport pipe 10 of the present embodiment, the flow path cross-section in the processing chamber internal transport section 10b and the flow path cross-section at the ejection end 10a are both circular with the same flow path cross-sectional area A1. According to this aerosol transport pipe 10, the aerosol is fed from the aerosol generating section 6, and the fed aerosol is ejected from the opening of the ejection end 10a.

Next, the flow path cross-sectional area A1 at the ejection end 10a of the aerosol transport pipe 10, a distance Ia between the ejection end 10a of the aerosol transport pipe 10 and the base material K, and the relationship between the flow path cross-sectional area A1 and the distance Ia will be explained.

The flow path cross-sectional area A1 of the ejection end 10a of the aerosol transport pipe 10 is not particularly limited as long as it is 10 mm² or more, but is preferably 20 mm² or more, more preferably 30 mm² or more, and even more preferably 95 mm² or more. Note that in the present embodiment, the flow path cross-sectional area A1 is 95 mm².

The distance Ia from the ejection end 10a of the aerosol transport pipe 10 to the base material K is not particularly limited, but is preferably 100 mm or less, more preferably 40 mm or less, and even more preferably 10 mm or less. On the other hand, if the distance between the ejection end 10a of the aerosol transport pipe 10 and the base material K is too small, when the base material K has a distorted shape, there is a risk that the ejection end 10a and the base material K will come into contact with each other when the aerosol transport pipe 10 and the base material K are moved relative to each other, and therefore it is preferable that the distance Ia between the ejection end 10a of the aerosol transport pipe 10 and the base material K is 2 mm or more. Note that in this embodiment, the distance Ia is 10 mm.

Also, with the film forming apparatus 1, the value obtained by dividing the flow path cross-sectional area A1 at the ejection end 10a of the aerosol transport pipe 10 by a square of the distance Ia between the ejection end 10a of the aerosol transport pipe 10 and the base material K (hereinafter referred to as "(A1/Ia²) value") is set to be 0.001 or more (that is, 95/10²=0.95 in the present embodiment). Note that although there is no particular limitation on the (A1/Ia²) value, it is preferably 0.001 or more, more preferably 0.007 or more, and even more preferably 0.03 or more. Also, the (A1/Ia²) value is preferably 25 or less, and more preferably 1 or less.

The carrier gas feeding means 15 includes a gas supply section 16, a carrier gas pressure control unit 17, a carrier gas flow rate control unit 18, a carrier gas feeding pipe S2, and the like.

Specifically, a carrier gas feeding pipe S2 is connected to the gas supply section 16, and the gas supply section 16 supplies gases such as air, N₂, He, and Ar to the carrier gas feeding pipe S2 using a compressor or a gas cylinder.

In this embodiment, the carrier gas feeding pipe S2 is for feeding the gas supplied from the gas supply section 16 to the aerosol generating section 6 as the carrier gas. Specifically, in the present embodiment, the gas sent from the gas supply section 16 is fed as the carrier gas to the aerosol generating section 6 via the carrier gas pressure control unit 17 and the carrier gas flow rate control unit 18 in the stated order, and the carrier gas feeding pipe S2 is constituted by a plurality of pipes connected between the gas supply section 16, the carrier gas pressure control unit 17, the carrier gas flow rate control unit 18, and the aerosol generating section 6.
Also, a pressure sensor P1 for detecting the pressure in the carrier gas feeding pipe S2 is provided between the carrier gas flow rate control unit 18 and the aerosol generating section 6 in the carrier gas feeding pipe S2.

The carrier gas pressure control unit 17 statically stabilizes the carrier gas flowing through the carrier gas feeding pipe S2 at an appropriate pressure, and the carrier gas flow rate control unit 18 controls the flow rate of the carrier gas flowing through the carrier gas feeding pipe S2. In this embodiment, the operations of the carrier gas pressure control unit 17 and the carrier gas flow rate control unit 18 are appropriately controlled based on the pressure detected by the pressure sensor P1 and the like.

### Ceramic Raw Material Powder

Particles constituting the ceramic raw material powder used in the film forming apparatus 1 preferably have a density of 4.0 g/cm³ or more, and such particles include, for example, particles of stabilized zirconia in which yttrium, calcium, magnesium, hafnium, or the like is contained in zirconia. Note that in this embodiment, yttrium-containing zirconia (YSZ) is used as the ceramic raw material powder.

### Film Formation Method

Next, the process of forming a film (formed film) on the base material K through the film forming method using the film forming apparatus 1 will be described. In the film forming method according to the present embodiment, the carrier gas is supplied from the gas supply section 16 to the aerosol generating section 6 while the carrier gas pressure control unit 17 and the carrier gas flow rate control unit 18 adjust the flow rate and pressure of the carrier gas flowing through the carrier gas feeding pipe S2. The aerosol generating section 6 generates an aerosol in which the fed carrier gas and the ceramic raw material powder supplied from the raw material powder supply section 7 are mixed. The generated aerosol is fed to the aerosol transport pipe 10.

The aerosol fed to the aerosol transport pipe 10 is ejected from the ejection end 10a of the aerosol transport pipe 10 toward the base material K, and the ejected aerosol collides with the base material K to form a film on the base material K.

Here, the aerosol ejected toward the base material K is ejected from the ejection end 10a having a circular flow path cross section, and the above (A1/Ia²) value is 0.95 (that is, 0.001 or more). Accordingly, the ejected aerosol has a uniform speed in the flow path cross section of the ejection end 10a, and variation in particle speed in the direction perpendicular to the base material K at the time of collision with the base material K is less likely to occur. For this reason, adhesion of a powder compact and formation of porosity are suppressed, and a homogeneous and dense film is formed. In particular, when the ceramic raw material powder is a stabilized zirconia such as YSZ, which has a relatively high density, a highly dense and homogeneous film can be formed. In addition, since the flow path cross-sectional area A1 of the ejection end 10a is 95 mm² (i.e., 10 mm² or more), the ceramic raw material powder is less likely to accumulate at the ejection end 10a, and a large amount of ceramic raw material powder can be stably supplied for a long time, and therefore it is possible to form a film on the base material K over a long period of time.

Working Examples 1 to 5 and Comparative Examples 1 to 4 will be described below. Film formation was performed for a predetermined time while moving the base material back and forth along a predetermined direction with different shapes of the flow path cross-section at the ejection end of the aerosol transport pipe, different flow path cross-sectional areas, and different distances between the ejection end and the base material. YSZ particles having a density of 5.9 g/cm³ and a median diameter of 1.01 µm were used as the raw ceramic powder in each of the working examples and comparative examples. Also, the flow rate of the carrier gas was set to 18 L/min, and the pressure in the processing chamber was set to 0.2 kPa in each working example and each comparative example.

Tables 1 to 3 are tables summarizing various conditions and results for Working Examples 1 to 5 and Comparative Examples 1 to 4, and "area of porous region" in Table 2 shows the area of a porous region with a low adhesive strength.
Also, FIG. 4 is a diagram showing the ejection end of the nozzle used in Comparative Example 1, and the area of the A3 portion indicated by shading in FIG. 4 is the flow path cross-sectional area. The shape of the nozzle used in Comparative Example 1 is a shape conventionally adopted as the shape of the nozzle of an apparatus for performing film formation processing through the AD method.
Furthermore, FIG. 5 is a diagram showing the ejection end of the nozzle used in Comparative Example 2, and the area of the A2 portion indicated by shading in FIG. 5 is the flow path cross-sectional area. FIG. 6 is a diagram schematically showing the base material after the film formation processing in Comparative Example 1, and the up-down direction in FIG. 6 is the movement direction of the base material. Also, FIG. 7 is a diagram schematically showing the base material after the film forming processing in Comparative Example 2, and, similarly to the above, the up-down direction in FIG. 7 is the movement direction of the base material. Note that in FIGS. 6 and 7, the dark shaded portions are the portions where a powder compact is adhered.

**[Table 1]**

| | Work. Ex. 1 | Work. Ex. 2 | Comp. Ex. 1 | Comp. Ex. 2 |
|---|---|---|---|---|
| Flow path cross-sectional shape | Circular (11 mm φ) | Circular (11 mm φ) | Slit-shaped (10 mm × 0.6 mm) | Square (10 mm square) |
| Flow path cross-sectional area (mm²) | 95 | 95 | 6 | 100 |
| Distance between ejection end and base material (mm) | 10 | 40 | 10 | 10 |
| (A1/Ia²) value | 0.950 | 0.059 | 0.060 | 1 |
| Adhesion state of powder compact | Not adhered | Not adhered | Adhered | Adhered |

**[Table 2]**

| | Work. Ex. 3 | Work. Ex. 4 | Work. Ex. 5 |
|---|---|---|---|
| Flow path cross-sectional shape | Circular (5.5 mm φ) | Circular (5.5 mm φ) | Circular (5.5 mm φ) |
| Flow path cross-sectional area (mm²) | 23.75 | 23.75 | 23.75 |
| Distance between ejection end and base material (mm) | 10 | 40 | 60 |
| (A1/Ia²) value | 0.237 | 0.015 | 0.007 |
| Area of porous region (mm²) | 56 | 336 | 364 |
| Adhesion state of powder compact | Not adhered | Not adhered | Not adhered |

**[Table 3]**

| | Comp. Ex. 3 | Comp. Ex. 4 |
|---|---|---|
| Flow path cross-sectional shape | Circular (2.25 mm φ) | Circular (2.25 mm φ) |
| Flow path cross-sectional shape (mm²) | 3.97 | 3.97 |
| Distance between ejection end and base material (mm) | 10 | 5 |
| (A1/Ia²) value | 0.040 | 0.159 |
| Adhesion state of powder compact | Adhered | Adhered |

As can be understood from Table 1, when comparing Working Examples 1 and 2 with Comparative Examples 1 and 2, no adhesion of the powder compact was observed in Working Examples 1 and 2, whereas a large amount of powder compact was adhered in Comparative Examples 1 and 2 (see FIGS. 6 and 7). For example, as shown in FIG. 7, in Comparative Example 2, when the film formation processing is performed while the base material is moved back and forth, a large amount of the powder compact is adhered to the portion where the particles in the aerosol sprayed toward the base material from the corner portion where the flow of the aerosol is likely to be disturbed. Based on these findings, it was confirmed that by making the cross-sectional shape of the ejection end of the aerosol transport path circular instead of square or slit-shaped as in the conventional technique, the flow speed of the aerosol becomes uniform within the flow path cross-section, and a uniform film can be formed on the base material.

Also, as shown in Table 2, even in Working Examples 3 to 5, in which the cross-sectional areas of the flow paths are slightly smaller than those in Working Examples 1 and 2, adhesion of the powder compact is not observed. On the other hand, regarding Working Examples 3 to 5, when the area of the porous region is focused on, it can be understood that the area of the porous region decreases and the uniformity of the film improves the higher the (A1/Ia²) value is.

Also, as shown in Table 3, in Comparative Examples 3 and 4, in which the cross-sectional areas of the flow paths are smaller than those of Working Examples 3 to 5, a large amount of the powder compact was adhered to the base material even though the cross-sectional shape of the flow path was circular. It is assumed that this is because even if the cross-sectional shape of the flow path is circular, the raw material powder will be clogged if the cross-sectional area of the flow path is too small. Due to this, it was confirmed that even if the channel cross-sectional shape is circular, a flow path cross-sectional area of a certain degree is required in order to suppress the formation of the powder compact and form a homogeneous film on the base material, and if the flow path cross-sectional area is too small, a homogeneous film cannot be formed on the base material.

Due to the above, it was confirmed that, as in the film forming apparatus 1 and the film forming method according to the present embodiment, by using an aerosol transport pipe 10 in which the flow path cross-section at the ejection end 10a is circular with an area of 10 mm² or more, a large amount of ceramic raw material powder can be stably supplied for a long time, and a homogeneous film can be formed.

### Other Embodiments

[1] In the above embodiment, the flow path cross-sectional area A1 at the ejection end 10a of the aerosol transport pipe 10 was 10 mm² or more, and the (A1/Ia²) value was 0.001 or more, but there is no limitation to this. If the flow path cross-sectional area A1 is 10 mm² or more, the (A1/Ia²) value does not need to be 0.001 or more.
[2] In the above embodiment, the distance from the ejection end 10a of the aerosol transport pipe 10 to the base material K was 100 mm or less, but there is no limitation to this as long as the flow path cross-sectional area A1 is 10 mm² or more. In particular, if the cross-sectional area A1 of the flow path is 10 mm² or more and the (A1/Ia²) value is 0.001 or more, variation in the particle speed in the direction perpendicular to the base material at the time of collision with the base material is less likely to occur, and therefore the effect of suppressing adhesion of a powder compact and formation of porosity is obtained.
[3] In the above embodiment, the aerosol transport pipe 10 was a cylindrical straight pipe member, but there is no limitation to this. Even if a crushing mechanism for crushing aggregated particles, a classifying mechanism for classifying particles, or the like is separately provided in the path of the straight pipe member, the flowability of the aerosol is not impaired, and therefore it is possible to stably supply a large amount of ceramic raw material powder for a long time. As long as the shape of the flow path cross-section at the ejection end 10a of the aerosol transport tube 10 is substantially circular, the straight tube member need not be used. Note that the substantially circular shape includes not only a perfect circle but also an elliptical shape. The substantially circular shape also includes triangles and polygons with curved corners, the polygons having a number of corners greater than or equal to that of a pentagon, and quadrilaterals with curved corners in which the ratio (r/R) of a radius r of a curved surface portion of a corner of the quadrilateral and the radius R of a circumscribing circle exceeds 0.3. In such a case as well, the flow speed of the aerosol at the ejection end becomes uniform within the cross section of the flow path, and therefore the effect of forming a homogeneous and dense film on the base material can be obtained.
[4] In the above embodiment, the flow path cross-section at the processing chamber internal transport section 10b of the aerosol transport pipe 10 and the flow path cross-section at the ejection end 10a were both circular with the same flow path cross-sectional area A1, but there is no limitation to this, and the shapes of both flow path cross-sections may be different from each other. For example, the shape of the flow path cross-section at the ejection end 10a may be circular, and the shape of the flow path cross-section at the processing chamber internal transport section 10b need not be circular, and the shapes of both flow path cross-sections may both be circular and have different areas. Note that the area of the flow path cross-section in the processing chamber internal transport section 10b of the aerosol transport pipe 10 is preferably 10 mm² or more, more preferably 20 mm² or more, more preferably 30 mm² or more, and even more preferably 95 mm² or more.
[5] In the above embodiment, the processing chamber was depressurized to 0.6 kPa or less, but the present invention is not limited to this.

### Industrial Applicability

The present invention can be applied to a film forming apparatus and film forming method for forming a film on a base material, and a formed film.

### Description of Reference Signs

- 1: Film forming apparatus
- 10: Aerosol transport pipe (aerosol transport path)
- 10a: Ejection end
- 10b: Processing chamber internal transport section
- K: Base material

## Claims

1. A film forming apparatus (1) for forming a film on a base material (K), comprising
a processing chamber (2) with an inner space in which the base material (K) is arranged by a holding section (5),
a raw material powder supply section (7) configured to supply a ceramic raw powder,
an aerosol generating section (6) configured to generate an aerosol by dispersing the ceramic raw material powder in gas, and
an aerosol transport path suitable for ejecting an aerosol obtained by dispersing the ceramic raw material powder in a gas, from an ejection end (10a) toward the base material (K),
wherein the ejection end (10a) is disposed in the processing chamber (2), and the ejection end (10a) is opposed the holding section (5),
wherein an end portion opposite to the ejection end (10a) is connected to the aerosol generating section (6),
wherein a flow path cross-section at the ejection end (10a) of the aerosol transport path has a circular shape with an area of 10 mm² or more, the processing chamber (2) with an inner space in which at least a portion on a side of the ejection end (10a) of the aerosol transport path and the base material (K) are arranged,
wherein a flow path cross-section of the aerosol transport path at a processing chamber (2) internal transport section located in the processing chamber (2) has the circular shape with an area of 10 mm² or more,
wherein the shape of the flow path cross-section at the processing chamber (2) internal transport section corresponds to the shape of the flow path cross-section at the ejection end (10a), and
wherein the aerosol transport path is constituted by a straight pipe member.

2. The film forming apparatus (1) according to claim 1,
wherein the processing chamber (2) is depressurized to include a pressure of 0.6 kPa or less by discharging gas by a mechanical booster pump (3) and a vacuum pump (4) serving as exhaust equipment.

3. A film forming method using a film forming apparatus (1) according to claim 1 or 2.

4. The film forming method according to claim 3,
wherein a density of particles constituting the ceramic raw material powder is 4.0 g/cm³ or more.

5. The film forming method according to claim 3 or 4,
wherein the ceramic raw material powder is stabilized zirconia.

## Patentansprüche

1. Filmbildungseinrichtung (1) zur Bildung eines Films auf einem Basismaterial (K), umfassend
eine Verarbeitungskammer (2) mit einem Innenraum, in dem das Basismaterial (K) durch einen Halteabschnitt (5) angeordnet ist,
einen Rohmaterialpulverzuführabschnitt (7), der zum Zuführen eines keramischen Rohpulvers konfiguriert ist,
einen Aerosolerzeugungsabschnitt (6), der konfiguriert ist, um durch Dispergieren des keramischen Rohmaterialpulvers in Gas ein Aerosol zu erzeugen, und
einen Aerosoltransportpfad, der geeignet ist, ein durch Dispergieren des keramischen Rohmaterialpulvers in ein Gas erhaltenes Aerosol von einem Ausstoßende (10a) in Richtung des Basismaterials (K) auszustoßen,
wobei das Ausstoßende (10a) in der Verarbeitungskammer (2) angeordnet ist, und das Ausstoßende (10a) Halteabschnitt (5) gegenüberliegt,
wobei ein dem Ausstoßende (10a) gegenüberliegender Endabschnitt mit dem Aerosolerzeugungsabschnitt (6) verbunden ist,
wobei ein Strömungspfadquerschnitt am Ausstoßende (10a) des Aerosoltransportpfades eine kreisförmige Form mit einer Fläche von 10 mm² oder mehr aufweist, wobei die Verarbeitungskammer (2) einen Innenraum aufweist, in dem zumindest ein Abschnitt auf einer Seite des Ausstoßendes (10a) des Aerosoltransportpfades und das Basismaterial (K) angeordnet sind,
wobei ein Strömungspfadquerschnitt des Aerosoltransportpfades in einem in der Verarbeitungskammer (2) angeordneten inneren Transportabschnitt der Verarbeitungskammer (2) eine kreisförmige Form mit einer Fläche von 10 mm² oder mehr aufweist,
wobei die Form des Strömungspfadquerschnitts im inneren Transportabschnitt der Verarbeitungskammer (2) der Form des Strömungspfadquerschnitts am Ausstoßende (10a) entspricht, und
wobei der Aerosoltransportpfad aus einem geraden Rohrelement besteht.

2. Filmbildungseinrichtung (1) nach Anspruch 1,
wobei die Verarbeitungskammer (2) durch Ablassen von Gas durch eine mechanische Druckerhöhungspumpe (3) und eine Vakuumpumpe (4), die als Absaugeinrichtung dienen, so druckentlastet wird, dass sie einen Druck von 0,6 kPa oder weniger einschließt.

3. Filmbildungsverfahren unter Verwendung einer Filmbildungseinrichtung (1) nach Anspruch 1 oder 2.

4. Filmbildungsverfahren nach Anspruch 3,
wobei eine Dichte der Teilchen, aus denen das keramische Rohmaterialpulver besteht, 4,0 g/cm³ oder mehr beträgt.

5. Filmbildungsverfahren nach Anspruch 3 oder 4,
wobei das keramische Rohmaterialpulver stabilisiertes Zirkonoxid ist.

## Revendications

1. Appareil de formation de film (1) pour former un film sur un matériau de base (K), comprenant
une chambre de traitement (2) avec un espace intérieur dans lequel le matériau de base (K) est agencé par une section de maintien (5),
une section de fourniture de poudre de matière première (7) configurée pour fournir une poudre de matière première céramique,
une section de génération d'aérosol (6) configurée pour générer un aérosol en dispersant la poudre de matière première céramique dans un gaz, et
un chemin de transport d'aérosol approprié pour éjecter un aérosol obtenu en dispersant la poudre de matière première céramique dans un gaz, depuis une extrémité d'éjection (10a) vers le matériau de base (K),
dans lequel l'extrémité d'éjection (10a) est disposée dans la chambre de traitement (2), et l'extrémité d'éjection (10a) est opposée à la section de maintien (5),
dans lequel une partie d'extrémité opposée à l'extrémité d'éjection (10a) est reliée à la section de génération d'aérosol (6),
dans lequel une section transversale de chemin d'écoulement à l'extrémité d'éjection (10a) du chemin de transport d'aérosol présente une forme circulaire avec une surface de 10 mm² ou plus, la chambre de traitement (2) avec un espace intérieur dans lequel au moins une partie sur un côté de l'extrémité d'éjection (10a) du chemin de transport d'aérosol et le matériau de base (K) sont agencés,
dans lequel une section transversale de chemin d'écoulement du chemin de transport d'aérosol au niveau d'une section de transport interne de chambre de traitement (2) située dans la chambre de traitement (2) présente la forme circulaire avec une surface de 10 mm² ou plus,
dans lequel la forme de la section transversale de chemin d'écoulement au niveau de la section de transport interne de chambre de traitement (2) correspond à la forme de la section transversale de chemin d'écoulement à l'extrémité d'éjection (10a), et
dans lequel le chemin de transport d'aérosol est constitué d'un élément tuyau droit.

2. Appareil de formation de film (1) selon la revendication 1,
dans lequel la chambre de traitement (2) est dépressurisée pour inclure une pression de 0,6 kPa ou moins en évacuant du gaz au moyen d'une pompe basse pression mécanique (3) et d'une pompe à vide (4) servant d'équipement d'échappement.

3. Procédé de formation de film utilisant un appareil de formation de film (1) selon la revendication 1 ou 2.

4. Procédé de formation de film selon la revendication 3,
dans lequel une densité de particules constituant la poudre de matière première céramique est de 4,0 g/cm³ ou plus.

5. Procédé de formation de film selon la revendication 3 ou 4,
dans lequel la poudre de matière première céramique est de la zircone stabilisée.
